

# UNITED STATES PATENT OFFICE.

WILLIAM JAMES CORDNER, OF LONDON, ENGLAND, ASSIGNOR TO LOUIS D. BRANDEIS, TRUSTEE, OF BOSTON, MASSACHUSETTS.

## COMPOSITION OF MATTER.

SPECIFICATION forming part of Letters Patent No. 655,169, dated July 31, 1900.

Application filed February 6, 1900, Serial No. 4,194. (No specimens.)

To all whom it may concern:

Be it known that I, WILLIAM JAMES CORDNER, a subject of the Queen of Great Britain and Ireland, residing at London, England, 5 have invented a certain new and Improved Composition of Matter, (for which I have made application for Letters Patent in Great Britain under No. 20,934, dated October 19, 1899,) of which the following is a specification.

10 The object of this invention is the synthetic production of india-rubber by the assimilation of kindred gums and fibers, which under certain conditions appear to have a natural affinity for each other and yield in the after- 15 production an elastic material possessing the qualities of natural rubber.

In carrying out my invention I take china-grass or rhea fiber, which I have previously desiccated to remove any oil or volatile matter therefrom, and the latex of the *Tabernaemontana crassa* in or about the proportions hereinafter mentioned. I thoroughly incorporate these materials by feeding them in between a pair of hot rolls at a temperature 25 of about 120° Fahrenheit and work the materials until they are thoroughly incorporated. I then place the mixed materials in an oven, the temperature of which is about 300° Fahrenheit. The oven heat is gradually raised 30 to a temperature between 350° Fahrenheit and 400° Fahrenheit. The whole time of the working operation will be about four hours, and I find that the required combination will take place if during the last two 35 hours of the process a temperature of about 360° Fahrenheit is maintained. The mass thus formed is then allowed to cool, when on examination it will be found that although the fibrous structure of the rhea or other

40 similar fiber remains its textile strength has completely broken down. The material is then worked at a temperature of about 120° Fahrenheit through mixing-rolls until its fibrous structure has disappeared and the 45 whole is reduced to a uniform mass. During this latter treatment oxygen-giving substances are introduced, such as borate of manganese, permanganate of potassium, or a curing agent, such as sulfur, to the extent 50 of five to eight per cent., and, if desired, a toughening material, such as balata, to the extent of about ten per cent., may be added to give strength to the resultant product.

The mass is then allowed to rest for about forty-eight hours for the purpose of what 55 might be termed "synthetic digestion" or "assimilation." It is then placed in a suitable vessel inside a steam-chest and subjected to steam-heat at a pressure of forty to forty-five pounds to the square inch, the pressure being 60 gradually raised from nil until the working pressure is reached, the time allowed for raising being about one hour. This pressure is kept up for one to two hours and then allowed to fall back to zero, when the material 65 should be removed and allowed to cool. This completes the synthesis, and the resultant product possesses all the qualities of india-rubber. From this stage it can be worked the same as cleaned rubber and loaded up in 70 accordance with the purpose for which it is intended.

I have found from experience the following proportions to give excellent results for various grades of material:

75

|              | Formulae.                                                                                                           | Product.                                                                                  |
|--------------|---------------------------------------------------------------------------------------------------------------------|-------------------------------------------------------------------------------------------|
| Class I...   | Latex ..... 80 per cent.<br>Rhea fiber ..... 15 per cent.<br>Sulfur ..... 5 per cent.                               | A flexible material similar to that known in the trade as "dough." This is a cheap grade. |
| Class II...  | Latex ..... 72 per cent.<br>Rhea ..... 10 per cent.<br>Balata ..... 10 per cent.<br>Sulfur ..... 8 per cent.        | A similar material to Class I, but of a higher grade.                                     |
| Class III... | Latex ..... 75 per cent.<br>Rhea ..... 20 per cent.<br>Sulfur ..... 5 per cent.                                     | A flexible material like Class I for making up into hard goods like vulcanite.            |
| Class IV...  | Latex ..... 80 per cent.<br>Rhea ..... 15 per cent.<br>Permanganate of potassium or borate of manganese 5 per cent. | A material similar in every respect to Class I.                                           |

80

85

90

What I claim as my invention, and desire 95 to secure by Letters Patent, is—

A composition of matter consisting of china-grass or rhea fiber and the latex of the *Tabernaemontana crassa*, substantially as described.

In witness whereof I have hereunto set my 100 hand in presence of two witnesses.

WILLIAM JAMES CORDNER.

Witnesses:

REGINALD WILLIAM JAMES,  
RICHARD A. HOFFMANN.